

Oct. 27, 1936.

J. W. SPARKS

2,059,051

ROAD OILS

Filed Dec. 29, 1932



INVENTOR

Joseph W. Sparks  
BY  
Donald E. Payne  
ATTORNEY

## UNITED STATES PATENT OFFICE

2,059,051

## ROAD OILS

Joseph W. Sparks, Hammond, Ind., assignor to  
 Standard Oil Company, Chicago, Ill., a corpora-  
 tion of Indiana

Application December 29, 1932, Serial No. 649,430

5 Claims. (Cl. 196—22)

This invention relates to road oils, and it per-  
 tains more particularly to the process of treating  
 road oils to improve their desirable character-  
 istics.

5 Road oils must conform to very strict specifi-  
 cations, prescribed by State highway departments  
 for oils used on public roads. Usually these oils  
 must contain at least 6% of material insoluble in  
 hexane, they must not contain more than a prede-  
 10 termined amount of volatile matter, they must  
 have a minimum percentage of material insoluble  
 in carbon disulfide, they must yield a certain con-  
 tent of 100° F. melting point residue, and the as-  
 phaltic residue must have a high ductility. It is  
 15 often difficult, if not impossible, to meet road oil  
 specifications by merely fractionating the crude  
 mixed base or asphaltic base petroleum oil, and  
 it is likewise difficult or impossible to meet the  
 road oil specifications with fractions or blends of  
 20 "pressure tar" (tar obtained by cracking, polymer-  
 izing, or hydrogenating petroleum products to  
 form gasoline, etc.). The object of my invention is  
 to provide a means for treating pressure tar or  
 25 similar carbonaceous materials obtained from  
 petroleum whereby it can be made to meet the  
 rigorous road oil specifications. More particular-  
 ly, the object is to increase the hexane insoluble  
 material of road oil without materially affecting  
 30 its other characteristics.

I accomplish the desired result by lightly  
 chlorinating the road oil with a gas in which the  
 chlorine is diluted and in which the amount of  
 chlorine is maintained within critical limits.  
 Heretofore it has been generally supposed that the  
 35 addition of chlorine to liquid hydrocarbons of this  
 sort would result in the formation of a sludge and  
 grainy carbon-like particles which would separate  
 from the oil. It was believed that the chlorina-  
 tion would raise the carbon disulfide insoluble  
 40 content to a very considerable extent. I have  
 discovered that when small amounts of chlorine  
 diluted with air are added in small quantities at  
 comparatively low temperatures to road oils, the  
 hexane insoluble content thereof is raised very  
 45 materially without materially affecting the other  
 properties. I have discovered that it is important  
 to control the amount of chlorine employed to  
 give the maximum hexane insoluble material.  
 The percentage of hexane insoluble material can  
 50 be increased about 65% to 70% by the use of  
 critical amounts of chlorine between 0.05% to 0.1%  
 and 1.0%, the maximum effectiveness being ob-  
 tained by the use of about 0.4%. The results ob-  
 tained are decidedly unexpected from two points  
 55 of view; first, that minute quantities of chlorine

have such a pronounced effect in raising the  
 hexane insoluble content of the road oil and sec-  
 ond, that no sludges or other products are formed  
 which are insoluble in the oil or in carbon di-  
 sulfide. Furthermore, the product is quite non-  
 5 corrosive, and can be stored in iron containers for  
 long periods of time without attack on the metal.

The invention will be more clearly understood  
 from the following detailed description and from  
 the accompanying drawing which forms a part 10  
 of this specification and in which—

Figure 1 represents diagrammatically an ele-  
 vation of my chlorination system;

Figure 2 is a graph showing the effect of the  
 amount of chlorine added on the amount of 15  
 hexane insoluble material produced; and

Figure 3 is a graph showing the effect of added  
 chlorine on the viscosity of the road oil.

I will describe my invention as applied to a road  
 oil prepared from pressure tar obtained from the  
 cracking of Mid-Continent gas oil. This pres-  
 sure tar has a hexane insoluble content of 3.8%,  
 an evaporation loss of 6.7%, an asphalt content  
 of 44.0%, a furol viscosity at 77° F. of 86 seconds,  
 and a carbon disulfide soluble content of 99.8%. 25  
 It should be understood, however, that the inven-  
 tion is applicable to road oils of widely varying  
 characteristics and from varying sources, par-  
 ticularly road oils which are deficient in the per-  
 centage of hexane insoluble material. 30

The road oil can be stored in a suitable storage  
 tank 10 and heated by means of steam coils 11 to  
 a temperature of about 150° F. to about 180° F.  
 Although this is the preferred temperature for my  
 treatment, the chlorination can be done at any 35  
 reasonable temperature from 80-300° F., as long  
 as the chlorine is sufficiently diluted, as will be  
 hereinafter described.

Chlorine gas from high pressure cylinder 12 is  
 metered through valve 13 and mixed with about 40  
 ten volumes of air from storage tank 14. The air  
 may be compressed by compressor 15 and it may  
 be metered through valve 16 to line 17, wherein  
 it is mixed with chlorine. The dilute chlorine is  
 conducted by pipe 17 to an injector or diffuser, 45  
 such as perforated pipe 18, and an amount of  
 chlorine gas is blown into the road oil equal to  
 about 0.4% by weight thereof. The relative pro-  
 portions of chlorine and diluent gas are not criti-  
 cal and will depend somewhat on the tempera- 50  
 tures employed. At high dilutions there may be  
 an objectionable loss of unreacted chlorine and at  
 low dilutions there may be an immediate forma-  
 tion of insoluble matter at the locus of the chlorine  
 bubble. Previous attempts at straight chlorina- 55

tion have probably resulted in sludge formation because the concentration of the chlorine was too high at the temperatures employed or because too much chlorine was employed. The reaction of 5 the chlorine is a vigorous one and even at a 1-10 dilution, no free chlorine is found in the exit gases. However, large quantities of hydrogen sulfide and hydrogen chloride are given off through vent 18. The finished product may be 10 withdrawn from feed line 20 after the above described reaction.

The precise amount of chlorine and the exact dilution can be varied somewhat with different road oils, but one skilled in the art can base the 15 reaction on the preferred embodiment hereinabove described.

By adding dilute chlorine gas in small increments in the manner hereinabove described I have found that the percentage of hexane insoluble material varies as shown in Figure 2 and that for this particular stock the optimum results are obtained by the use of 0.4% of chlorine (by weight). In Figure 3 I have shown the effect of the added chlorine on viscosity. It appears 25 that no other characteristic of the road oil is materially changed; the evaporation loss, asphalt content and amount of material soluble in carbon disulfide all check the original untreated road oil within the limits of experimental error.

30 I have described the use of air as a diluent but it should be understood that I can use other gases for this purpose. I prefer to use an oxidizing gas because I believe it supplements the action of the chlorine. I prefer to use about 10 35 volumes of air per volume of chlorine but I can use from one to twenty volumes or even larger amounts under various operating conditions and with various road oils. A simple test will show whether or not the concentration of chlorine is 40 sufficiently high to cause sludge formation and sufficient diluent should be used to avoid sludging.

While I have described in detail a preferred embodiment of my invention it should be understood that I do not limit myself to said details except as defined by the following claims, which should be construed as broadly as the prior art will permit.

I claim:

50 1. The method of treating pressure tar to convert it into a satisfactory road oil which comprises contacting said pressure tar at a temperature of about 80° F. to about 300° F. with from

about 0.05% to about 1.0% of its weight of chlorine gas, said chlorine gas being diluted with at least about an equal volume of a diluent gas such as air, whereby the hexane insoluble content of said pressure tar is increased without materially 5 affecting the other properties thereof.

2. The method of treating pressure tar to convert it into a satisfactory road oil which comprises contacting said pressure tar at a temperature of about 150° F. to about 180° F. with from 10 about 0.05% to about 1.0% of its weight of chlorine gas, said chlorine gas being diluted with at least about an equal volume of a diluent gas such as air, whereby the hexane insoluble content of said pressure tar is increased without materially 15 affecting the other properties thereof.

3. The method of treating pressure tar to convert it into satisfactory road oil which comprises injecting a dilute chlorine gas into a body of said pressure tar maintained at a temperature of 20 about 80° F. to about 300° F., the chlorine gas being diluted with at least about an equal volume of air, the total amount of chlorine being limited to about 0.05% to about 1.0% by weight based on 25 said pressure tar, whereby the hexane insoluble content of said pressure tar is increased without materially affecting the other properties thereof.

4. The method of treating pressure tar to convert it into a satisfactory road oil which comprises injecting dilute chlorine gas into a body of 30 said pressure tar maintained at a temperature of about 80° F. to about 300° F., the chlorine gas being diluted with about 1 to about 20 volumes of a diluent gas such as air, the total amount of 35 chlorine being limited to about 0.1 to about 1.0% by weight based on said pressure tar, whereby the hexane insoluble content of the pressure tar is increased without materially affecting the other properties thereof.

5. The method of treating pressure tar to convert it into a satisfactory road oil which comprises injecting dilute chlorine gas into a body of 40 said pressure tar maintained at a temperature of about 80° F. to about 300° F., the chlorine gas being diluted with about 1 to about 20 volumes of 45 a diluent gas such as air, the total amount of chlorine being limited to about 0.4% by weight based on said pressure tar, whereby the hexane insoluble content of said pressure tar is increased without materially affecting the other properties 50 thereof.

JOSEPH W. SPARKS.